

## 1

3,745,120

## NON-CORROSIVE SULFUR-LIQUID HYDROCARBON SLURRY CONTAINING AN ASPHALTENIC COMPOUND

Mary Frances Vondrak, Houston, Tex., assignor to Shell Oil Company, New York, N.Y.

No Drawing, Continuation-in-part of application Ser. No. 772,008, Oct. 30, 1968, now Patent No. 3,597,005.

This application Feb. 19, 1971, Ser. No. 117,127

Int. Cl. B01j 13/00; C09k 3/00

U.S. Cl. 252—309

4 Claims

## ABSTRACT OF THE DISCLOSURE

An improved non-corrosive sulfur-liquid hydrocarbon slurry composition and method of preparing said slurry for transportation in suitable vehicles such as pipelines without causing plugging and corrosion.

## CROSS-REFERENCE

This is a continuation-in-part of copending patent application Ser. No. 772,008, filed Oct. 30, 1968, now U.S. Pat. 3,597,005.

## FIELD OF THE INVENTION

The invention relates to a new, improved and novel non-corrosive, non-plugging sulfur-liquid hydrocarbon slurry composition having incorporated therein a small amount of an aqueous solution containing an asphaltic material, said slurry composition being particularly designed for transportation through conduits such as pipelines or vehicles such as tankers, etc.

## BACKGROUND OF THE INVENTION

The invention relates to a new, improved and novel non-slurry in pipelines is well known in the art as noted by reference to U.S. Pats. 2,798,772; 2,917,345 or 2,947,578 or as described in Pipeline Industry, June 1967, pp. 58-60 or Chem. Eng. Prog., vol. 61, No. 2, 72, 1965. In forming a sulfur-hydrocarbon slurry, the sulfur is generally sprayed in molten form into either water or a hydrocarbon in an amount sufficient to form a slurry suitable for transportation through a pipeline. Formation of a stable noncorrosive sulfur-containing slurry wherein the sulfur does not undergo any undesirable change or the slurry does not exhibit a tendency to wide variation in viscosity is essential to the process in addition to other problems which may be encountered during and after transportation of the slurry through a pipeline. Thus, separation of the sulfur from the carrier fluid results in plating or coating of the sulfur vessel walls, e.g. pipeline walls causing corrosion and plugging of the pipeline. Viscosity changes in the slurry due to pressure and temperature variations encountered under such conditions results in increase in pumping power which increases operation costs, etc. These are a few of the problems normally encountered and which must be avoided in transporting sulfur-liquid hydrocarbon slurries through pipelines or other vehicles. However, a most troublesome one is that of corrosion encountered in the preparation, transportation, and recovery of such slurry systems for if excessive corrosion is encountered in any of these three phases then the slurry system cannot be put into operation.

Although these are serious problems for consideration in the preparation and transportation and recovery of sulfur, nevertheless if the corrosion problem is controlled, it can be made to be an effective and economically attractive means of preparing and transporting such slurries particularly since sulfur is normally recovered or obtained from isolated, remote and inaccessible areas. As noted above, a number of methods have been proposed

## 2

for pipeline transportation of sulfur slurries such as by injecting molten sulfur into water or a liquid hydrocarbon thereby forming a sulfur slurry for pipeline transportation. Such means for preparing and transporting sulfur do not overcome the corrosion, coating or plugging problems described above.

An object of the present invention is to prepare for transport sulfur as a sulfur-liquid hydrocarbon slurry composition which is non-corrosive, stable and flowable.

Another object of the present invention is to transport through a pipeline sulfur-liquid hydrocarbon slurries without causing sulfur coating, deposition or plugging or corrosion of the pipeline.

Still another object of this invention is to form a slurry

15 of sulfur in a liquid hydrocarbon medium, which when formed is stable, non-corrosive, does not tend to cause pipeline plugging when said slurry is transported through a pipeline and from which the sulfur can be readily recovered as essentially pure sulfur.

20 Another object is to transfer sulfur as a liquid hydrocarbon slurry by pipeline over great distances reducing pumping and handling costs.

Other objects will be apparent from the following description.

## 25 SUMMARY OF THE INVENTION

The invention relates to a new, improved and novel non-corrosive, non-plugging sulfur-liquid hydrocarbon slurry composition containing therein a small amount

30 of an aqueous solution containing a nitrogen organic compound having at least one amino or amino-amide or imidazole group in the molecule, said slurry composition being particularly designed for transportation through conduits such as pipelines or vehicles such as tankers, etc.

35 Specifically, the present invention is directed to an improved, novel and new technique for preparing for vehicle transportation such as pipeline transportation of a sulfur-liquid hydrocarbon slurry through pipelines over great distances without causing corrosion, coating, deposition or

40 plugging of the pipeline due to the tendency of sulfur under such conditions to adhere to the pipeline walls because of temperature, pressure and other variable conditions to corrode and plug said lines; by admixing or adding or injecting prior to or after injection of a sulfur-liquid hydrocarbon slurry into the pipeline, a small amount of 0.1 to 10% by weight, preferably between about 0.5 to about 5% by weight, of an aqueous solution

45 basis total slurry and from about 20 to about 5000 p.p.m. basis oil phase of an asphaltic material extracted from crude oil by any suitable means or an asphalt containing 20 to about 5000 p.p.m. basis oil phase of asphaltic material. Asphaltenes can include materials described in

50 "The Chemical Constituents of Petroleum"—Sachanen, Chapter 9 and include petroleum resins, asphaltenes, asphaltogenic acids their derivatives and mixtures thereof and include materials described in the Journal of the Institute of Petroleum, April 1968, pages 107-114 and February 1968, pages 50-53 or as described in U.S. Pats. 3,275,076; 3,284,340; or 3,336,146 and these materials can be separated from petroleums by methods described in U.S. Pats. 3,364,138 and 3,368,876. The asphaltenes as defined should be present in the final mixture in an amount preferably not exceeding 2000 p.p.m. basis oil phase and the additive can be injected when necessary in various places along the pipeline where indications are that corrosion or plugging of the line might take place.

55 Any corrosion and plugging detection means known in the art can be used for this purpose. It has been noted that by injection of 1-5% by weight of an aqueous solution basis total slurry and a small amount (20-2000 p.p.m. basis oil phase of an asphaltene as defined into a pipeline transporting a sulfur-liquid hydro-

60 65 70

carbon slurry in which the sulfur content of the slurry can vary from about 10% by weight sulfur, inhibits corrosion and prevents plugging of 30 and 70% by weight sulfur, inhibits corrosion and prevents plugging of the line due to sulfur deposition on the walls of the pipeline, resulting in improved flow of the slurry at reduced pumping cost. A preferred plugging and corrosion preventing composition for sulfur-liquid hydrocarbon slurries being pipeline transported is the addition to such slurries of from about 1 to 5% by weight water basis total slurry and 20-2000 p.p.m. basis oil phase of an asphaltenic material selected from the group consisting of asphalt, asphaltenes, asphaltogenic acid and mixtures thereof.

The sulfur-liquid hydrocarbon slurry can be made by any suitable means such as described in U.S. Pat. 2,798,772, or 3,443,837. It is preferred that methods for making the sulfur-liquid hydrocarbon slurry be used in which the sulfur is produced in spherical form since this facilitates the stable dispersion and suspension of the sulfur in the liquid hydrocarbon carrier and inhibits attrition and reduces friction. The phase transfer method for making the sulfur slurry as described in the above copending application comprises first forming a sulfur-aqueous liquid (water) slurry and thereafter phase transferring the sulfur particles from the aqueous liquid into a liquid hydrocarbon. In this process the phase transformation to form the sulfur-hydrocarbon slurry can be so controlled that a small amount (1-5% by weight) water basis total slurry is transferred with the sulfur-water phase into the hydrocarbon phase and thereafter an asphaltenic material can be added to accomplish the desired ends of the present invention. Slurries thus prepared contain sulfur in particle form of 5-5000 microns, preferably 30-350 microns and are spherical in shape.

The hydrocarbon carrier for the sulfur can be any liquid hydrocarbon ranging from a light petroleum fraction such as liquefied petroleum gas (LPG), fuel oil, gasoline, kerosene, petroleum distillates condensates, crude oil and mixtures thereof. Preferred are liquid hydrocarbons containing at least 10% by weight or higher of aromatics, preferably about 15-30% by weight aromatic enriched kerosene or crude oil or crude oil condensate fractions containing 15-20% by weight aromatics which include mono- and polycyclic aromatic hydrocarbons.

At the terminal end of the line the aqueous solution can be readily separated from the sulfur-hydrocarbon system by suitable phase separation, distillation or the like.

#### PREFERRED EMBODIMENT OF THE INVENTION

40-60% by weight sulfur in (a) aromatic (17% by weight) enriched kerosene or (b) a petroleum condensate or (c) a blend of (b) and crude oil slurries, were prepared by phase transfer by first injecting molten sulfur into an aqueous liquid such as water and thereafter contacting the slurry thus formed with hydrocarbons (a), (b) or (c) to effect phase transfer of the sulfur particles into the hydrocarbon, and injecting this slurry into a pipeline followed by injection of 2% by weight water basis oil phase and about 20-800 p.p.m. basis oil phase of an asphaltene additive shown in Table 2. Sulfur-hydrocarbon slurries thus formed in the presence of the water and an asphaltene additive of the present invention do not corrode or plug pipelines. Instead of using the phase transfer technique for making the slurry, the molten sulfur can be injected in the hydrocarbons (a), (b) or (c) directly and thereafter admixed with the aqueous solution and additive.

An advantage of the present process for transporting through pipelines sulfur-liquid hydrocarbon slurries is that the slurry can be also prepared by directed injection of molten sulfur into a suitable liquid hydrocarbon as described in U.S. Pat. 2,798,772 and injecting therein a small amount of water and an asphaltene additive so

as to prevent corrosion and plugging of the line. Either process as well as other processes can be used to make the sulfur-liquid hydrocarbon slurry depending on the availability of the liquid carriers. Thus, where water is available the first process can be used and if not, the second one can be used.

The corrosive effect of added or adventitious water on sulfur-liquid hydrocarbon slurries is evident from the data presented in Table 1 and the selectiveness and unexpected effect of asphaltenic additives of this invention as corrosion preventive agents is shown in Table 2.

The slurry tested comprised 40% by weight sulfur and 60% hydrocarbon and the conditions for the corrosion test were as follows:

#### CORROSION BY SULFUR SLURRIES

##### Conditions:

15 150 ml. magnesia bottles rotated at 10 r.p.m. in EPR bottle rotator.  
 20 120 grams of slurry added to each bottle. Slurry concentration=40% w. sulfur.  
 25 Sulfur particle size: Jumping Pound sulfur 81% greater than 45 microns. Waterton sulfur 82% greater than 45 microns.  
 Oil phase: Kerosene with aromatics.  
 30 Water additions are percent by weight of the oil fraction.  
 1/2 x 6 1/8-inch specimens of 20-gauge mild steel sheet with sandblasted surface.  
 Specimens wedged into bottles to reduce mechanical damage.  
 Room temperature (72°), atm. pressure, 48 hours exposure.

TABLE 1

#### Sulfur slurry corrosion as a function of water concentration

Conditions: As above. 40% w. Waterton sulfur/kerosene with 17% w. aromatics.

| Water concentration, percent w. <sup>a</sup> : | Corrosion rate, mils./yr. <sup>b</sup> |
|------------------------------------------------|----------------------------------------|
| 0                                              | 1                                      |
| 0.28                                           | 50                                     |
| 1.12                                           | 120                                    |
| 2.2                                            | 230                                    |
| 4.4                                            | 250                                    |
| 5.0                                            | 280                                    |

<sup>a</sup> Concentration of added water, basis oil.

<sup>b</sup> From weight loss and exposure time. Corrosion rates have not been corrected for weight loss due to cleaning.

TABLE 2

#### Effect of asphaltenes on sulfur slurry corrosion

55 Conditions: As in Table 1. 40% w. Jumping Pound sulfur/kerosene with aromatics plus 2% w. H<sub>2</sub>O (basis oil).

| Additive c:                                                | Corrosion rate, mpy. <sup>a</sup> |
|------------------------------------------------------------|-----------------------------------|
| Medicine River Crude Asphaltenes b 210 p.p.m.              | 8.8                               |
| 0.1 percent w.                                             | 5                                 |
| Asphalt 0.061 percent w. containing 170 p.p.m. asphaltenes | 4.5                               |

<sup>a</sup> From weight loss and exposure time. Corrosion rates have not been corrected for weight loss due to cleaning.

<sup>b</sup> Produced by heptane precipitation.

<sup>c</sup> Additives are basis oil phase.

At the terminal end of the line the water phase can be readily removed by phase separation and the sulfur can be removed from the liquid hydrocarbon by suitable means such as described in U.S. Pat. 2,798,772 and the sulfur, purified by methods as described in U.S. Pats. 2,809,885 and 3,489,671 which latter patent teaches treating oil contaminated sulfur with an aqueous solution containing a mixture of alkali hydrosulfide and corresponding hydroxide, e.g., ammonium hydrosulfide and ammonium hydroxide, or by other suitable means such

as sulfur can be recovered from the oil slurry by filtration of molten sulfur and liquid-liquid extraction with a hydrocarbon solvent containing 10-50% by weight aromatic. Thus, at the receiving terminal the sulfur slurry can be filtered and washed. The recovered sulfur is then melted and purified by liquid-liquid extraction with an aromatic hydrocarbon such as cumene. Also, if desired, the filtered sulfur can be steam stripped to recover bright yellow sulfur.

The foregoing description of the invention is merely intended to be explanatory thereof. Various changes in the details of the described method may be made within the scope of the appended claims without departing from the spirit of the invention.

I claim as my invention:

1. A method of preparing a sulfur-liquid hydrocarbon slurry composition and inhibiting the undesired corrosive effects of the slurry on pipeline walls comprising spraying at least 10% of molten sulfur into a liquid hydrocarbon and thereafter admixing therein a small amount of from 0.1% to 10% of an aqueous solution containing from about 20 to about 5000 p.p.m. basis oil phase of an asphaltenic compound extracted from crude oil.

2. The method of claim 1 wherein the liquid hydrocarbon is petroleum oil and the asphaltenic compound is asphalene.

3. The method of claim 2 wherein the oil is crude oil.

5

4. A method of preparing a sulfur-liquid hydrocarbon slurry composition and inhibiting the undesired corrosive effects of the slurry on pipeline walls comprising spraying from about 10% to about 75% of molten sulfur into a liquid hydrocarbon and thereafter admixing therein a small amount of from 0.1% to 10% of an aqueous solution containing from about 20 to about 5000 p.p.m. basis hydrocarbon phase of an asphalene.

10

#### References Cited

##### UNITED STATES PATENTS

|           |        |           |       |         |
|-----------|--------|-----------|-------|---------|
| 2,343,860 | 3/1944 | Bencowitz | ----- | 252-31  |
| 2,204,967 | 6/1940 | Moser     | ----- | 252-8.3 |

15

##### FOREIGN PATENTS

|         |        |               |       |        |
|---------|--------|---------------|-------|--------|
| 129,132 | 7/1919 | Great Britain | ----- | 252-31 |
|---------|--------|---------------|-------|--------|

20

##### OTHER REFERENCES

Chemical Abstracts, vol. 55, col. 21554b.  
Chemical Abstracts, vol. 46, col. 2785i and vol. 59, col. 12564f.

25

JOHN D. WELSH, Primary Examiner

U.S. CL. X.R.  
252-388, 393, 45; 302-66